

April 30, 1935.

H. I. SHAW ET AL

1,999,790

PROCESS FOR HARDENING GRAY AND MOTTLED CAST IRON

Filed Aug. 18, 1930

**FIG. 1.**



**FIG. 2.**



**FIG. 3.**



INVENTORS

Howard I. Shaw  
Newton S. Hoerle

BY *Lancaster, Allwin and Rommel*  
ATTORNEYS.

## UNITED STATES PATENT OFFICE

1,999,790

PROCESS FOR HARDENING GRAY AND  
MOTTLED CAST IRONHoward I. Shaw and Newton S. Hoerle,  
Muskegon, Mich.

Application August 18, 1930, Serial No. 476,164

3 Claims. (Cl. 148—3)

This invention relates to improvements in processes or methods for the hardening of gray and mottled cast iron.

The primary object of the invention is the provision of an improved method for the production of cast iron parts, such as valve tappets and cam shafts, which will materially harden the cast iron parts during formation, to produce the necessary physical properties and wear resisting, strengthening, and toughening characteristics which will permit of the economical, durable and efficient formation and use of the parts.

In the drawing, forming a part of this specification:

15 Figure 1 is a view in elevation of a valve tappet in a mould, portions of the mould being in vertical section.

Figure 2 is a view in elevation of the cast iron tappet removed from the mould.

20 Figure 3 is a similar view of the finished valve tappet, partly in elevation and partly in section to show characteristics thereof.

While the invention is particularly directed to the provision of a durable and economically produced one-piece cast iron valve tappet, yet the method is not to be limited to the provision of such parts.

We may use ordinary gray or mottled cast iron of conventional composition in the cupola and if desired may have suitable alloys to increase wear resisting and other qualities and properties. We have found that good results are obtained by using a composition consisting of:

Cupola charge—

35 20% steel  
40% pig iron  
40% foundry return scrap

Ladle additions—

1 3/4 # ferro molybdenum  
40 1/2 # ferro vanadium

Analysis of ferro vanadium—

37.90% contained

Analysis of ferro molybdenum—

57% contained

45 Since the analysis of constituents of the cast iron have influence on the physical properties and hardness, we do not restrict ourselves to the above formula. Indeed, we have used a higher per cent of steel scrap than that listed in the cupola charge, and the percentage of vanadium varies between .15 and .25%. The alloy additions may or may not be used, as desired.

The molten iron, at a temperature ranging from 2500° F. to 2700° F. is poured from the cupola 50 into sand moulds, shown at 10 in Figure 1 of the

drawing. The mould chamber 11 in this case is shaped to form a valve tappet 12 consisting of a disc-shaped head 13 and an integral shank or stem 14, as shown in the drawing. The molten iron is chilled at the time of pouring, using conventional cast iron chill plates or the like. In the specific instance a chill plate 15 is provided, upon which the head 13 may be formed, for the purpose of chilling and hardening the same. The depth of the chill plate can of course be varied.

5 Other means may be provided for chilling the cast iron as it is poured into the mould, such as the use of a metallic mould kept cool by circulation of water or the like. This chilling operation is used to produce extreme and localized hardness, particularly in the head portion of the specific tappet shown. The depth of the chill can of course be varied within limits. The chilled portion of the article is hardened to a state or constituent known as cementite, which is of course 10 iron carbide. This gives the extreme wear resisting qualities to the article, which are so essential in the case of a tappet head.

15 Next, the casting, after it has solidified in the mould and dropped to a temperature below 700° F. may be removed, although the casting from the mould may be removed at any time after it has cooled sufficiently and it is then quickly heated in a suitable furnace to a temperature ranging between 1550° F. and 1700° F. preferably to a 20 temperature of 1650° F. which we have found to be best. The statement that the casting is to be heated quickly means that the cast iron article should not be held at the temperatures above set forth for any great length of time, since by so 25 doing would break up the combined carbon or cementite into ferrite and graphite. Therefore the heating of the article after casting is very carefully carried out, preferably by heating the furnace previous to introduction of the article 30 to 1650° F. When the article is placed in the furnace the temperature in the furnace, due to the cold casting, will naturally drop. The castings are heated to a temperature of 1650° 35 F. as quickly as possible, and when the furnace has again reached the desired temperature, preferably 1650° F. the castings are removed and quenched in oil, water, or any other suitable quenching medium. The castings are permitted 40 to remain in the quenching bath until cold, or until the castings have reached the same temperature as the quenching medium. The temperature of the quenching bath preferably ranges 45 from 100 to 110° F. The heating and quenching produces a very uniform structure and uniform

5

10

15

20

25

30

35

40

45

50

55

hardness, probably caused by the fact that some of the carbon is thrown back into solid solution with the iron and held therein thru the cooling stage during quenching. A uniform martensitic-troostitic structure is produced with a corresponding hardness of approximately 600 Brinell, which structure can be broken down to a sorbitic-pearlitic structure and corresponding decrease of hardness by regulating the time and temperature of heating at the time of drawing the temper.

After the quenching operation the castings are "drawn" to relieve internal strains produced during the quenching operation. The immediate step after quenching is to place the castings in a furnace and heat them to approximately 500° to 600° F. holding them approximately one hour for each inch of cross section of the article. For a valve tappet, fifteen to twenty minutes will suffice. This temperature reduces the hardness somewhat; relieving internal strains caused by quenching, and it should be borne in mind that the temperature of re-heating must be regulated according to the hardness desired.

If desired, the chilling of the iron during moulding may be eliminated, since the subsequent steps will produce a very uniform structure, with resulting uniform hardness throughout the article cast. In normal gray cast iron there is an uneven distribution of carbons. However, with our improved heat treatment, a very uniform structure is produced, having a uniform distribution of carbon. This particularly applies to castings of uneven tension; eliminating soft and weak spots in the casting, and giving greater hardness with increased physical properties, and especially giving better wear-resisting qualities and greater strength and toughness. This refers particularly to iron which has not been chilled, and if desired the chilling step may be included to render particular parts of the casting harder than others, for instance, the head in the particular tappet shown. The casting shown, when it comes from the mould, will have a Brinell hardness of around 180 to 200 on the unchilled portion. The subsequent heating and quenching will raise the hardness to from 400 to 450 Brinell. On the chilled head or section, however, the Brinell hardness will be approximately 600.

As before noted the addition of alloys, such as the use of approximately 1% molybdenum will materially improve the physical properties and wear resisting qualities of the casting.

In order to bring out the importance of the invention it should be noted that cast iron parts hardened by means of chilling alone have certain inherent defects, namely, brittleness, lack of controlled hardness and strength. In the case of chilled tappets, which are not subject to the heating and quenching steps as mentioned herein, the stem is too soft and gauls where the tappet

bearing is disposed; the threads strip, and the heads are too brittle, very often breaking in service. Therefore, it can readily be understood that the specific heat treatment, quenching and drawing of our invention produces a casting which is tough, durable, wear-resistant and hard without resulting brittleness.

It should be noted that the castings are left in the mould until they are black, or at the temperature above mentioned, and after taking out they are rough-machined before heating to 1650° F.

Various changes in the steps of the method and process herein outlined, and the application of the same to the formation of various articles and parts may be made to the invention herein shown and described, without departing from the spirit of the invention or the scope of the claims.

We claim:

1. The steps in the method of treating cast iron which consists in chilling the cast iron at the time of pouring to produce an extreme localized hardness, quickly heat treating the cast iron after removal from the mould to a temperature of substantially 1650° F., said heat treating at 25 said temperature continuing over a period of time sufficient to increase the hardness of the unchilled portion and insufficient to soften and reduce the hardness of the chilled portion, said period being considerably less than one hour, 30 and quenching the then heated parts in a quenching bath.

2. The method of producing cast iron valve tappets, having a hardened head portion and a relatively softer stem, which consists in casting 35 the valve tappet and chilling the head portion of the tappet at the time of pouring to produce an extreme localized hardness there, subsequently quickly heat treating the cast tappet to approximately 1650° F., for a sufficient time to materially 40 harden the unhardened portion of said tappet said last mentioned time being insufficient to affect the chilled head portion materially, and immediately thereafter quenching the casting.

3. Those steps in the method of producing a 45 chilled cast iron article which consists in treating a casting having a Brinell hardness of between 180 to 200 of a portion of said casting and a Brinell hardness substantially greater of another portion of said casting, by subjecting said casting 50 to a temperature of substantially 1650° F., bringing said casting to substantially said temperature and immediately quenching said casting, whereby the hardness of the softer portion is raised to substantially 450 Brinell and a hardness of substantially 600 Brinell is maintained by the harder portion.

HOWARD I. SHAW.  
NEWTON S. HOERLE.